

# United States Patent Office

3,314,793

Patented Apr. 18, 1967

1

3,314,793

## NON-DIFFUSING INHIBITORS OF FORM- ALDEHYDE HARDDENING

Kenneth C. Kennard and Hyman L. Cohen, Rochester, N.Y., assignors to Eastman Kodak Company, Rochester, N.Y., a corporation of New Jersey  
No Drawing. Filed Dec. 27, 1962, Ser. No. 247,524  
8 Claims. (Cl. 96—83)

This invention relates to gelatin compositions containing non-diffusing inhibitors of hardening by formaldehyde which are polymers containing a hydrocarbon backbone and having a group like



as a substituent therein.

In the use of gelatin particularly for photographic products for forming layers therein formaldehyde has been added to increase the resistance of the gelatin layer to swelling by water. Formaldehyde has been found to act rapidly and efficiently for this purpose. However, formaldehyde as a hardener has the disadvantage that it will migrate from the layer in which it has been incorporated to adjacent layers. This has been found undesirable in photographic products having a plurality of gelatin layers, some of which layers should be hardened and others retained in a non-hardened condition. This is particularly true in products for use in photographic products which depend on the stripping of one layer from another. Also in paper manufacture, sizing materials are sometimes used which may release formaldehyde. When gelatin layers are applied to paper of this nature there is the danger of migration of formaldehyde from the paper base to gelatin layers applied thereover.

One object of our invention is to provide gelatin compositions in which the hardening effect of formaldehyde which migrates thereto is inhibited. Another object of our invention is to provide gelatin compositions containing polymeric materials which will inhibit the hardening effect of formaldehyde on the gelatin therein which materials will not diffuse or migrate therefrom to other adjacent layers. A further object of our invention is to provide photographic products having gelatin layers hardened by means of formaldehyde plus other layers in less hardened or unhardened condition. A still further object of our invention is to provide gelatin compositions which contain polymeric materials composed of a hydrocarbon backbone and having



or the like as a substituent group therein. Other objects of our invention will appear herein.

We have found that gelatin compositions containing polymeric materials having a hydrocarbon backbone and a substituent



group, R<sub>1</sub>, R<sub>2</sub> and R<sub>3</sub> being hydrogen, alkyl, hydroxyalkyl and the like, no substituent having more than 20 carbon atoms, will resist or partially resist the hardening effects of formaldehyde. We have found that these gelatin compositions may be employed for the application of layers in photographic products, which layers resist the hardening effect from formaldehyde which might migrate thereto either from the use of formaldehyde as a hardener in an adjacent layer or from paper stock in which a formaldehyde releasing material has been used in the preparation of the paper. We have found that photo-

2

graphic products may be prepared having a plurality of layers on a support in which the gelatin layers containing polymeric materials as defined herein remain in an unhardened condition even though formaldehyde or formaldehyde-forming compounds are present in adjacent layers. We have found that by incorporating certain polymeric materials in gelatin layers the use of formaldehyde as a hardener for gelatin in adjacent layers is made possible without experiencing any hardening effect upon the gelatin layers in which the certain polymers have been incorporated. We have found that by the use of lesser amounts of the polymeric material the hardening effect of formaldehyde may be lessened, in cases where complete resistance to formaldehyde hardening is not desired.

In its broadest aspects our invention comprises gelatin compositions containing polymers having a hydrocarbon backbone and a substituent



group, R<sub>1</sub>, R<sub>2</sub> and R<sub>3</sub> being hydrogen, alkyl, hydroxyalkyl and the like, no substituent having more than 20 carbon atoms. Our invention includes gelatin layers containing these materials and photographic products composed of layers containing formaldehyde or formaldehyde-forming compounds and gelatin layers in which polymeric materials having a hydrocarbon backbone and



as a substituent group are present therein.

Polymeric materials having a hydrocarbon backbone and a substituent



group, R<sub>1</sub>, R<sub>2</sub> and R<sub>3</sub> being hydrogen, alkyl, hydroxyalkyl and the like, no substituent having more than 20 carbon atoms, adapted for use in preparing compositions in accordance with our invention are illustrated by the following compounds which have been found to be particularly useful for preparing gelatin coating compositions and gelatin layers: poly(4-vinylsemicarbazide), poly(acrylic hydrazide), copoly(vinyl acetate-maleic hydrazide), poly(vinyl-N-carbhydrazoyl methyl carbamate), poly(acrylic semicarbazide), poly(1-methyl-4-vinyl semicarbazide) and poly(1-beta-hydroxyethyl-4-vinyl semicarbazide). These compounds when present in any proportion in a gelatin composition exhibit an inhibiting effect against hardening by formaldehyde. The most convenient proportions however are those found within the range of 2-20% based on the weight of the gelatin.

Gelatin compositions in accordance with our invention (1) may be used as carriers for silver halide in photographic emulsions such as where a photographic product having an unhardened emulsion layer is desired, (2) they may be used for the application of intermediate layers especially as a stripping layer for products employed in photographic processes involving the stripping of one layer from another, (3) they may be employed as the carrier for baryta in applying a baryta coating to paper, or (4) where a controlled lesser degree of hardening is desired accomplished by the use in the gelatin composition of a diminished amount of the inhibitor. The gelatin compositions in accordance with our invention are useful in any connection where an unhardened gelatin layer is desirable. As the inhibitors in accordance with our invention do not

migrate from the layer in which they were incorporated to adjacent layers compositions in accordance with our invention make possible the presence of formaldehyde hardened gelatin layers and unhardened gelatin layers in immediate contact with each other.

The following examples are of procedures for preparing inhibitors of formaldehyde hardening which are useful in preparing compositions in accordance with our invention:

*Example 1*

A solution of 268 grams of phenol in 375 ml. of dry ether was added dropwise over a period of one half hour to a stirred solution of 178 grams of vinyl isocyanate in 500 ml. of dry ether keeping the temperature at between 6 and 12° C. with external cooling. Following addition, the mixture was stored overnight in the refrigerator. The solution was then washed with 600 ml. of a 5% sodium hydroxide solution, dried and the solvent evaporated under vacuum. The residual solid was dissolved in a hot benzene ligroin solution and the mixture cooled. The precipitated solid was recrystallized from a benzene ligroin solution giving 315 grams of crystals in 75-76%.

70 grams of these crystals (N-vinyl phenyl carbamate) and 350 mg. of azobisisobutyronitrile were dissolved in 70 ml. of benzene and the mass was heated overnight on a 60° bath. The viscous solution obtained was diluted with acetone and precipitated in ether. Poly(N-vinyl phenyl carbamate) resulted in the form of a white powder.

32.6 grams of the poly(vinyl phenyl carbamate) thus obtained was mixed with 64 grams of anhydrous hydrazine and 36 grams of water and the mass was stirred for 3 hours on a 60° bath. Solution was complete except for a little gelatinous material. The solution was filtered and precipitated in methanol. The precipitate was vacuum dried forming a white powder for poly(vinyl semicarbazide).

*Analysis.*—C, 37.9%; H, 7.0%; N, 35.6%.

*Example 2*

Twenty grams of vinyl acetate-maleic anhydride interpolymer were added with stirring to 300 ml. of hydrazine hydrate. The mass stood for 30 minutes at room temperature whereupon it was heated on a steam bath for one hour. A smooth moderately viscous dope was obtained. This dope was cooled and poured in a fine stream into 3 liters of stirred absolute ethyl alcohol which contained 30 ml. of 30% aqueous NaOH. A friable precipitate was obtained. This precipitate was washed with alcohol and obtained. This precipitate was washed with alcohol and was redissolved in 150 ml. of distilled water. Added was slowly to this solution with stirring was 6 ml. of aqueous NaOH whereupon the solution was poured into 2 liters of absolute alcohol containing 30% aqueous NaOH. The precipitate was extracted with absolute ethyl alcohol until free of alkali and was dried in a vacuum desiccator. The product was the hydrazide of vinyl acetate-maleic anhydride interpolymer.

*Example 3*

21 grams of polymethyl acrylate, 96 grams of hydrazine and 54 grams of water was stirred at 60° for 4 hours. Most of the solid dissolved. The mass was diluted to one liter with water, filtered and dialyzed. The material remaining in the cellulose casing was evaporated to 300 ml. to contain 5% of solids. To obtain the dry product the mass was precipitated with methanol, and the precipitate was washed and vacuum dried to give dry polyacrylic hydrazide.

*Example 4*

A suspension was prepared of 10 grams of poly(N-vinyl O-phenyl carbamate) in 46 grams of N-methylhydrazine. The mass was tumbled overnight and was then heated for 3 hours on a steam pot. It was cooled, precipitated in ether and the precipitate was washed and vacuum dried. There was thus obtained 7.5 grams of poly[(1-methyl-4-

vinyl)semicarbazide] in the form of a white powder soluble in water. This material was found to be useful as an inhibitor of hardening of gelatin by formaldehyde. Also it did not migrate when placed in layers of gelatin adjacent to other layers of gelatin or other colloidal material.

*Analysis.*—C, 43.4%; H, 8.3%; N, 31.0%.

*Example 5*

10 grams of poly(N-vinyl-O-phenyl carbamate) was mixed with 76 grams of beta-hydroxyethylhydrazine. The mass was tumbled overnight forming a clear, very viscous solution. It was then heated for 3 hours on a 60° bath and the resulting mass was precipitated with n-propanol and the precipitate formed was repeatedly washed with propanol and vacuum dried. The polymer obtained was then dissolved in water, reprecipitated in propanol and vacuum dried. 5 grams of poly[(1-beta-hydroxyethyl-4-vinyl)-semicarbazide], soluble in water and in methanol was obtained.

*Example 6*

A mixture of 54 grams of N-bromosuccinimide, 2.3 grams of allyl chloride, 10 mg. of benzoyl peroxide and 500 ml. of chloroform was refluxed for 4 hours. After 25 cooling the mixture, there was added thereto 100 ml. of anhydrous methanol dropwise with stirring causing an exothermic reaction. After this addition the mixture was refluxed overnight. The solvent was evaporated off by vacuum and the residue obtained was recrystallized with 200 ml. of methanol giving 40 grams of N-(beta-bromoethyl)-O-methylcarbamate. 21 grams of the carbamate so prepared was dissolved in 100 ml. of acetonitrile and 10.2 grams of triethylamine was added thereto causing an exothermic reaction and the mixture was allowed to 30 stand for an hour and was then cooled whereupon crystals separated. The crystals were filtered off and the filtrate was poured into 500 ml. of ether. The precipitate thus formed was filtered off. The filtrate was evaporated to dryness under vacuum. The residue thus obtained was dissolved in 100 ml. of benzene and the mixture was 40 cooled to give 16 grams of crystals, melting at 138-140°, forming acrylyl methyl carbamate.

A solution was prepared of 20 grams of N,N-dimethyl acrylamide, 26 grams of acrylyl methyl carbamate and 45 0.5 gram of azobisisobutyronitrile in 100 ml. of acetone. The solution was heated overnight on a 50° bath under nitrogen. By morning the mixture had solidified. The polymer formed was dissolved in methanol and precipitated in ether which precipitate was washed and vacuum dried giving a white fibrous solid.

A mixture of 15 grams of the product obtained namely copoly(N,N-dimethyl acrylamide-N-acrylyl-O-methyl carbamate) and 300 ml. of hydrazine was tumbled overnight giving a clear, viscous solution. The mass was heated one hour in a 60° bath and the excess hydrazine was then removed under vacuum. The residue was dissolved in a mixture of 10 ml. of water and 200 ml. of methanol and was precipitated in ether. The precipitate was washed with isopropanol and dried. 13 grams of 55 copoly(acrylyl semicarbazide-N,N-dimethyl acrylamide) was obtained in a form of a white powder. This material was found to be a good inhibitor of gelatin hardening by formaldehyde and exhibited resistance to migration from gelatin layers, in which it was incorporated, to adjacent colloidal layers.

*Analysis.*—C, 46.6%; H, 7.8%; N, 22.8%.

The following examples illustrate the use of these inhibitors in gelatin compositions:

*Example A*

To a high speed silver bromoiodide gelatin emulsion formaldehyde was added. Non-diffusing inhibitor (polyacrylic hydrazide) as an aqueous solution, was added thereto just before coating. This emulsion was coated on a cellulose acetate support at a coverage of 1040 mg.

of gelatin per square foot and 460 mg. of silver per square foot. A sample of each coating was exposed on an Eastman Ib sensitometer, processed in Kodak DK-50 developer, fixed, washed, and dried. The tests of the various products including those without both formaldehyde and

## Example D

Procedure similar to that described in the preceding paragraphs was carried out using as the inhibitor poly(vinyl-N-carbhydrazoyl methyl carbamate). The results were as follows:

| Description              | Speed | $\gamma$ | Fog | Percent of Vertical Swell |                                         |
|--------------------------|-------|----------|-----|---------------------------|-----------------------------------------|
|                          |       |          |     | Freshly Coated            | 3-Day Incubation at 100° (Forced Aging) |
| 1. Control               | 100   | 1.32     | .11 | 1,008                     | 884                                     |
| 2. HCHO, 0.5% on wt. gel | 74    | .92      | .10 | 240                       | 221                                     |
| 3. 5% inhibitor          | 123   | 1.18     | .15 | 933                       | 820                                     |
| 4. 10% inhibitor         | 129   | 1.27     | .15 | 993                       | 893                                     |
| 5. #2 + #3               | 97    | 1.29     | .12 | 833                       | 763                                     |
| 6. #2 + #4               | 118   | 1.30     | .12 | 891                       | 807                                     |

inhibitor and those excluding one or the other gave the following results:

We claim:

1. A photographic product comprising a support con-

| Description                                  | Speed | $\gamma$ | Fog | Percent of Vertical Swell |
|----------------------------------------------|-------|----------|-----|---------------------------|
| 1. Control                                   | 100   | 1.07     | .11 | 658                       |
| 2. HCHO, 1% on wt. gel                       | 78    | .93      | .11 | 558                       |
| 3. HCHO, 3% on wt. gel                       | 74    | .80      | .09 | 264                       |
| 4. HCHO, 6% on wt. gel                       | 68    | .73      | .08 | 206                       |
| 5. Poly(acrylic hydrazide), 2.04% on wt. gel | 132   | .98      | .16 | 696                       |
| 6. #2 + #5                                   | 132   | .98      | .12 | 644                       |
| 7. #3 + #5                                   | 129   | 1.02     | .12 | 609                       |
| 8. #4 + #5                                   | 118   | .92      | .11 | 400                       |
| 9. Poly(acrylic hydrazide), 8.16% on wt. gel | 123   | .88      | .29 | 454                       |
| 10. #2 + #9                                  | 126   | .90      | .28 | 406                       |
| 11. #3 + #9                                  | 110   | .92      | .37 | 590                       |
| 12. #4 + #9                                  | 123   | .88      | .28 | 575                       |

## Example B

A similar procedure was employed as in the preceding paragraph except that copoly(vinyl acetate-maleic hydrazide) was used as the inhibitor. The results obtained were as follows:

40 taining thereon a gelatin layer having formaldehyde and adjacent thereto a non-hardened gelatin layer containing therein a formaldehyde hardening inhibitor comprising a

| Description                                                 | Speed | $\gamma$ | Fog | Percent of Vertical Swell |
|-------------------------------------------------------------|-------|----------|-----|---------------------------|
| 1. Control                                                  | 100   | 1.05     | .12 | 739                       |
| 2. HCHO, -3% on wt. gel                                     | 74    | .85      | .10 | 321                       |
| 3. HCHO, -6% on wt. gel                                     | 69    | .72      | .10 | 231                       |
| 4. Copoly(vinyl acetate-maleic hydrazide), 2.04% on wt. gel | 102   | 1.03     | .14 | 866                       |
| 5. #2 + #4                                                  | 89    | .90      | .11 | 387                       |
| 6. #3 + #4                                                  | 78    | .80      | .11 | 274                       |
| 7. Copoly(vinyl acetate-maleic hydrazide), 4.08% on wt. gel | 102   | 1.00     | .14 | 989                       |
| 8. #2 + #7                                                  | 102   | .98      | .13 | 662                       |
| 9. #3 + #7                                                  | 87    | .88      | .12 | 342                       |

## Example C

A similar procedure was used but poly(4-vinyl semicarbazide) was employed as the inhibitor. The results were as follows:

60 polymeric material having a hydrocarbon backbone and as a substituent group thereon:



| Description                               | Speed | $\gamma$ | Fog | Percent of Vertical Swell |
|-------------------------------------------|-------|----------|-----|---------------------------|
| 1. Control                                | 100   | 1.20     | .12 | 659                       |
| 2. HCHO, .5% on wt. gel                   | 76    | .87      | .10 | 240                       |
| 3. Polyvinyl semicarbazide 1% on wt. gel  | 110   | 1.58     | .11 | 651                       |
| 4. Polyvinyl semicarbazide 5% on wt. gel  | 110   | 1.41     | .10 | 574                       |
| 5. Polyvinyl semicarbazide 10% on wt. gel | 105   | 1.25     | .11 | 554                       |
| 6. #2 + #3                                | 83    | 1.02     | .10 | 267                       |
| 7. #2 + #4                                | 95    | 1.29     | .10 | 502                       |
| 8. #2 + #5                                | 95    | 1.32     | .10 | 569                       |

$R_1$ ,  $R_2$ , and  $R_3$  each being selected from the group consisting of hydrogen, alkyl and hydroxyalkyl.

2. A photographic product comprising a support having thereon a gelatin layer containing poly(4-vinyl semicarbazide) and thereover a silver halide gelatin photographic emulsion layer containing formaldehyde hardener.

3. A photographic product, some portion of which contains formaldehyde or a formaldehyde former, having therein a gelatin layer containing a formaldehyde hardening inhibitor comprising a polymeric material having a hydrocarbon backbone and as a substituent group thereon:



$R_1$ ,  $R_2$  and  $R_3$  each being selected from the group consisting of hydrogen, alkyl, and hydroxyalkyl.

4. A photographic product, some portion of which contains formaldehyde or a formaldehyde former, having therein a gelatin layer containing as a formaldehyde hardening inhibitor poly(4-vinyl semicarbazide).

5. A photographic product, some portion of which contains formaldehyde or a formaldehyde former, having therein a gelatin layer containing as a formaldehyde hardening inhibitor poly(acrylic hydrazide).

6. A photographic product, some portion of which

15

20

25

contains formaldehyde or a formaldehyde former, having therein a gelatin layer containing as a formaldehyde hardening inhibitor copoly(vinyl acetate-maleic hydrazide).

7. A photographic product, some portion of which contains formaldehyde or a formaldehyde former, having therein a gelatin layer containing as a formaldehyde hardening inhibitor poly(vinyl-N-carbhydrazoyl methyl carbamate).

8. A photographic product, some portion of which contains formaldehyde or a formaldehyde former, having therein a gelatin-silver halide photographic emulsion layer containing poly(4-vinyl semicarbazide).

#### References Cited by the Examiner

##### UNITED STATES PATENTS

|           |        |                 |        |
|-----------|--------|-----------------|--------|
| 2,668,154 | 2/1954 | Orth            | 260—6  |
| 2,940,956 | 6/1960 | Smith           | 96—114 |
| 3,168,400 | 2/1965 | Blackmer et al. | 96—22  |

##### OTHER REFERENCES

Kern et al.: Angew. Chem., vol. 69, pp. 153—71 (1957).  
Welzel et al.: Makromol. Chem., vol. 44—46, pp. 221—7 (1961).

NORMAN G. TORCHIN, Primary Examiner.

J. T. BROWN, R. H. SMITH, Assistant Examiners.